

# UNITED STATES PATENT OFFICE.

JACOUB AKTSCHOURIN, OF AKTSCHOURINSKI TUPIK, RUSSIA.

## PROCESS OF MAKING COLOPHONY AND COLOPHONY-SOAP.

1,074,339.

Specification of Letters Patent. Patented Sept. 30, 1913.

No Drawing.

Application filed October 24, 1911. Serial No. 656,505.

To all whom it may concern:

Be it known that I, JACOUB AKTSCHOURIN, a subject of the Czar of Russia, residing in Aktschourinski Tupik, on the Moscow-Kasan Railway, in the Empire of Russia, have invented certain new and useful Improvements in Processes of Making Colophony and Colophony-Sap, of which the following is a specification.

10 This invention relates to an improved process of making colophony and colophony-soap.

Heretofore colophony and soap from the same were made by subjecting pitch containing woods to the action of an alkali. These processes have the very objectionable disadvantage that they consume too much of the alkali in by-reactions, and that at the higher temperatures employed the alkali decomposes the incrusting substances or gums of the wood, by which substances the cells of the wood are held together. Besides the rosin-soap obtained has a dirty appearance and assumes due to the decomposition-products of the incrusting substances by the action of the alkali on the same, a disagreeable brown color.

The object of this process is to overcome these objections, and for this purpose the invention consists of a process of making colophony and colophony-soap by treating the shavings or other wooden bodies after distilling off the turpentine, with a diluted solution of an alkali under pressure and at a temperature below the boiling point of water and then separating the mixture of soap-glue and colophony-emulsion by mechanical means.

In carrying out the improved process, the wood is treated in the form of shavings, small pieces and the like, with the alkali-solution under pressure, but at a lower temperature than 100° C., as it was found that comparatively weak solutions of alkali did

not act on or decompose the incrusting or gummy substances of the wood. Besides, the alkali-solution converts the colophony under these conditions into an emulsion, without saponification, so that a considerably smaller quantity of alkali is necessary for the reaction than in the processes heretofore employed.

In the production of colophony and colophony-soap by the process mentioned, a diluted solution of an alkali is permitted to act on the shavings, etc.—after distilling the vapors of turpentine—while simultaneously the pressure in the still is raised to several atmospheres, care being taken that the boiling takes place at a temperature from 80 to 90° C. and at a pressure of from 2 to 3 atmospheres. Simultaneously the mixture is subjected to agitation in the still by suitable stirring means. After the process of saponification and the separation of the colophony has taken place, the liquor which is composed of a mixture of soap-glue and colophony-emulsion is thrown off from the shavings in a centrifugal machine.

70

I claim:

The process herein described of making rosin and rosin-soap from shavings of resinous woods, which consists in distilling off the turpentine from the shavings, then treating the shavings with a diluted solution of alkali under a pressure of from 2 to 3 atmospheres and at a temperature below 100° C., and separating the rosin-emulsion and soap-glue by mechanical means.

80

In testimony that I claim the foregoing as my invention, I have signed my name in presence of two subscribing witnesses.

JACOUB AKTSCHOURIN.

Witnesses:

DANIEL GARDNER,  
AUG. MICHIS.